

July 2, 1935.

E. WALTER

2,006,425

PROCESS FOR THE PRODUCTION OF CEMENTITIOUS MASSES

Filed Dec. 10, 1931

4 Sheets-Sheet 1



Fig. 1.



Fig. 2.



Fig. 3.



Fig. 4.



Fig. 5.



Fig. 6.



Fig. 7.

INVENTOR  
Ernest Walter  
BY  
John Specman  
his ATTORNEY

July 2, 1935.

E. WALTER

2,006,425

PROCESS FOR THE PRODUCTION OF CEMENTITIOUS MASSES

Filed Dec. 10, 1931 4 Sheets-Sheet 2

*Fig. 8.*



*Fig. 9.*



*Fig. 10*



*Fig. 11.*



*Fig. 13.*



INVENTOR

Ernest Walter  
BY  
Howard Freeman  
His ATTORNEY

July 2, 1935.

E. WALTER

2,006,425

PROCESS FOR THE PRODUCTION OF CEMENTITIOUS MASSES

Filed Dec. 10, 1931

4 Sheets-Sheet 3



Fig. 14.



Fig. 15.



Fig. 16.

INVENTOR  
Ernest Walter  
BY  
M. A. Henneberry  
his ATTORNEY

July 2, 1935.

E. WALTER

2,006,425

PROCESS FOR THE PRODUCTION OF CEMENTITIOUS MASSES

Filed Dec. 10, 1931

4 Sheets-Sheet 4



Fig. 17.

Fig. 18.



Fig. 20.

Fig. 19.

Fig. 21.



Fig. 22.



INVENTOR  
Fig. 23. Ernest Walter  
BY *Howard Spiegelman*  
his ATTORNEY

## UNITED STATES PATENT OFFICE

2,006,425

PROCESS FOR THE PRODUCTION OF  
CEMENTITIOUS MASSESErnest Walter, Montclair, N. J., assignor to Porete  
Mfg. Co., North Arlington, N. J., a corporation  
of New Jersey

Application December 10, 1931, Serial No. 580,994

13 Claims. (Cl. 25—155)

My invention relates to methods for treating cementitious materials to produce masses and forms thereof having the appearance of natural rocks and refers particularly to methods for producing such masses and forms as will be attractive and useful for making rock gardens and containers having the appearance of having been made from natural rocks.

In my invention I use, preferably, lightweight concrete for making the rocks because lightweight concrete is much lighter in weight, economic in handling and trucking, but mainly, because lightweight concrete is permeated by small air bubbles which makes the material much more attractive than solid concrete, having the appearance of pumice or coral rock, and is capable of holding considerable moisture which is so important for plants.

What I mean by lightweight concrete is not only concrete made with a lightweight aggregate, but aerated concrete made either by the foam method or by the metallic powder process which produces a gas, or any other lightweight concrete method by which the concrete is aerated.

All these lightweight concretes when they are ready to pour are of very liquid consistency—much more so than ordinary concrete.

It is very important that this lightweight concrete contain just the proper amount of water. This is much more essential than with the ordinary concrete. For ordinary concrete it does not matter so much whether it is mixed very dry or very wet, it will still give fairly good results. For instance, in ordinary concrete from as little as three (3) gallons of water per sack of cement can be used. The water contents of ordinary concrete mix can vary from above or as much as ten (10) gallons per sack. This means that twenty-five percent (25%) to eighty-five percent (85%) of water of the amount of cement can be used and the concrete will still be usable. This is entirely different for light concretes.

For instance, if the concrete is made with the foam method where we use approximately one-hundred (100) parts of Portland cement, one-hundred (100) parts of sand, about fifty (50) parts of water and three tenths part of foam compound and ten percent (10%) more water is used, the product will be too light and too weak and also the heavier particles of cement and sand will settle to the bottom before the concrete sets, which makes a product that is not uniform. If less water is used, say ten percent (10%) less, the mixture will collapse and it cannot be made very light in weight.

With the metal powder process where I use, for instance, one-hundred (100) parts of Portland cement, one-hundred (100) parts of sand, about fifty (50) parts of water and three tenths part of aluminum powder, if much water is used the heavier particles of the cement and sand are liable to settle the same as in the foam process. When the gas from the chemical reaction between the lime and cement and aluminum powder develops, this gas reaction is too rapid, the material raises higher and is liable to collapse afterward. If less water is used, the mixture will not rise at all, or very little and it is not possible to obtain a lightweight concrete.

I have found that by using ordinary soil or loam as a form material for my rocks, I can produce a very beautiful natural looking result. I take this soil or loam in the form of clumps or clods and pile it up rather loosely and irregularly into the proper shapes and then pour the lightweight concrete into moulds thus formed. On account of the very liquid consistency this concrete runs into all the interstices in the loosely piled pieces of soil, or loam. After the concrete is set, the soil or loam is removed by hand or other mechanical means and whatever cannot be thus removed easily is washed away with a water stream, which leaves the concrete in the original shape in which it was poured. I am aware that soil, dirt and loam have been used previously for casting concrete and other materials like cast iron, but for my purpose it is very important that this soil, or loam contains just the proper amount of water for moisture for the following reasons:—

If the soil is too dry it will absorb water from the lightweight concrete mixture.

If there is too much water in the soil, the lightweight concrete is liable to attract some of this water where it is in contact with the soil and the lightweight concrete mixture will behave as described above, that is, the heavier aggregates are liable to settle out and the concrete is liable to collapse before it sets, also if there is too much water in the soil, it is impossible to make the soil stand up in clumps with interstices between the clumps and it is not possible to get attractive appearing rocks.

For my purpose, I have found that with a certain kind of soil that I should have approximately twenty-five percent of water in the soil making attractive products.

If this particular soil material contains less than fifteen percent water, it will absorb so much water from the concrete mixture that the process

is not practical. If this soil material contains more than thirty-five percent water, it will not stand up properly and the concrete mixture is liable to take so much moisture from the soil material that it will not set properly as explained above. It can therefore be seen that it is very important to have the proper amount of water in this soil material.

Other soil, or materials, which I mention below 10 may require other percentages of water but in all cases the variation in the moisture contents of the forming material has to be small.

Another important property which the forming material should have is that it should be 15 easily removable from the deep pockets by a water stream. Ordinary clay or soil can be removed, but it takes considerable time and large amount of water under pressure to loosen it in the cavities and wash it out. The best material 20 to use for the purpose of washing out is sand. Very little water is required to wash sand out of deep holes, but sand alone is not always suitable because sand, if piled loosely, even if it is wet, will easily collapse and does not form hollow spaces in which the concrete should flow. For 25 many purposes I have found best to mix sand with a certain amount of clay, or ordinary soil, so as to get the right mixture. For some cases however, when no undercuts are required, sand 30 alone may be suitable. But in most cases when intricate undercut formations of the rocks are wanted, a mixture of soil and sand in varying proportions is better.

Instead of soil, or soil and sand, other materials 35 can be used, such as, sand and clay mixtures, diatomaceous earth, asbestos refuse, short fibred peat, fine crushed stone, slate powder, sawdust or any combinations of these and other suitable materials.

40 Instead of such mixtures of materials I can also use clumps made of plastic materials like soft rubber, gelatin, starch, glue, gluten, casein, gums and rosins as well as tar, asphaltic and other similar compounds.

45 These materials differ from those mentioned above in that instead of being made of a solid material and water so that they can be washed out of the cavities, they are made in lumps and of a viscous material which cannot be washed 50 out by water but it can be pulled out of the cavities. The plastic material of which these clumps can be made should have sufficient elasticity, strength and viscosity so that it can easily be removed from the cementitious material after 55 this is set and particularly so that these clumps can be pulled out of the cavities and hollows.

I am aware that some of these materials have 60 been used for the forming of objects made of cement and also plaster casts. It is common knowledge to use gelatin moulds which are usually made of gelatin, glycerine and some other ad-mixtures, or soft rubber forms for objects which have to be made in quantities of one or more. The new feature of my process for the use 65 of these plastics is the use of a great number of small and large clumps of all different shapes which are indiscriminately piled up or laid against a sheet wire mould. In this way they form an everchanging pattern for the cementitious material which runs into the interstices between these 70 clumps. Such plastic masses have the important property which is required for my process that they do not absorb any water from the cementitious materials nor do they add any water to it. After the cementitious materials are

set these clumps of plastic masses are removed and used over and over again.

In my specification and claims I refer to the above mentioned and other suitable materials as "soil".

Another feature of my invention is the following:

When a mould with wet soil is made, this soil is made so as to stand up almost vertically although usually it is advisable to give it an angle 10 of repose of about seventy-five degrees (75°). When the lightweight concentrate is poured into such a form, it will form a practically horizontal and flat surface on top which would not give us the irregular rocks that we desire to make.

15 In the accompanying drawings illustrating modified methods of following the process of my invention, similar parts are designated by similar numerals.

Figures 1 and 2 illustrate one method of following my process.

Figures 3 and 4 illustrate a modified method of following my process.

Figures 5, 6, and 7 illustrate a modified method of following my process.

Figures 8, 9, 10, 11 and 12, and 13 illustrate modified methods of following my process.

Figures 14 and 15 illustrate a modified method of following my process.

Figure 16 illustrates an arrangement of cementitious masses made by my process.

Figures 17, 18, 19, 20 and 21 illustrate a modified method of following my process.

Figures 22 and 23 illustrate a modified method of following my process.

One method of carrying out the process of my invention is shown in Figures 1 and 2, in which assembled clods or clumps of soil 10, 10, form a mould into which concrete 11 is poured to the level indicated in Figure 1. I then throw, or deposit, small clumps, or pieces, of soil 12, 12, upon the top surface of the concrete, preferably near the sides thereof.

This deposited soil raises the concrete level, and as the soil is usually somewhat heavier than the concrete, it sinks into the concrete, but not completely to the bottom, as shown in Figure 2. There is thus formed an irregularly shaped top portion to the concrete having a plurality of irregularly shaped pockets.

If the soil material thrown upon the top of the concrete mixture is too heavy, that is so heavy that it is liable to settle down to the bottom, it can be lightened in various ways, as for instance by mixing it with foam. Wet soil can be mixed with a foam made with the proper foaming materials and it can be made as light as the concrete mixture. In this way pieces of light soil can be incorporated into the mixture which practically float on the cement mixture.

When the metal powder process is used for 60 making lightweight concrete, the mixture rises after it is poured. During the rising of the mixture the clumps of soil can be inserted and many pockets can be provided. This metal powder process has the further advantage that the top 65 surface effects produced are similar to those of overflowing and cooling lava.

After the concrete sets, the soil material is removed by hand or a trowel or other mechanical means as well as possible, the remainder which is in the deep pockets is washed out by a powerful stream of water. The soil may be collected in a settling tank for re-use if desired. In order to save water, a pump can be used which circulates

the same water, from the settling tank to the nozzle which washes the rocks out.

The pockets which have been formed in the stones are very convenient for the planting of small plants which are usually used in rock and alpine gardens.

Figures 3 and 4 show another way for making rocks by my process. An irregular bed of soil 10, 10 is prepared on which clumps 10, 10, are set up on the same material to form hollow spaces in the rocks. The mixture of lightweight concrete 11 is then poured to the level as shown in Figure 3. Soil 12, 12, is thrown in the center so as to mark dividing lines between individual rocks. The concrete mixture will rise to a high and higher level and enough clumps of soil can be thrown in to make individual and irregular rocks.

Further pockets can be formed by waiting until the concrete is partially set and by throwing soil in clumps into this partially set concrete. Sand or fine dirt can also be thrown into the top which leaves an irregular speckled surface.

This invention applies not only to rocks but to whole rock mountains cast in large masses, also garden pools, Japanese gardens, bird baths, miniature mountains, sundials, benches, et cetera.

My process can also be applied for garden potteries. Figures 5, 6, and 7, for instance, show such garden pottery can be made. The soil is prepared on a flat surface as shown in Figure 5. The lightweight aerated concrete mixture is then poured to a determined level as to line X—X. Clumps of soil 12—12 are thrown into the sides which will raise the level of the concrete mixture as shown in Figure 6. Additional clumps of soil 13, 13 can be deposited so as to form natural pockets for the reception of small alpine and rock plants, or a core of soil material 14 can be inserted so as to make the desired size hole for plants. This makes a very attractive pattern. It is evident that these pots can be made in any desired shape and size.

My process can also be employed for making face building stone. This can be done either by the facing cast on the bottom or on the side or on the top. In all cases it is important that the forming material which is used has the right water contents. For instance, one method for making such blocks with the face on top is shown in Figures 8 and 9. The lightweight concrete mix 11 is poured into a square mould 15 as shown in Figure 8. After it is thus poured, soil material 12, 12 which can be lightened as explained above, is inserted upon the top of the concrete. After the concrete is set, this soil material is removed and washed off. If desired, such a faced material can be partially faced off as shown in Figure 10 which gives very beautiful effects.

Similar stone can be made not only for walls, but also for sidewalks, garden walks and floor slabs.

If the face of the blocks is made on the side, a square form 15 is made as shown on Figure 11 and then a soil material 12 inserted on the side as shown in Figure 12.

If the face of the blocks is produced on the bottom, this requires a similar mould as shown in Figure 13, the soil 12 being placed upon the bottom.

Figures 14 and 15 show another way for making pots. An open cylinder 16 is set up and soil 12 packed loosely against its outside. Concrete mixture 11 is then poured into the inside to a level Y—Y. Form cylinder 16 is then lifted up

about one half its height which will cause the mixture to run into the pockets of the loosely packed soil. At the same time a sandcore cylinder 17 is introduced from the top until it rests on precast chairs 18, 18, the cylinder 16 is then removed. The concrete mixture 11 rises and takes the shape shown in Figure 15. The soils 12 and 17 are washed away after the concrete is set, this produces a finished pot having an irregular outer face.

Figure 16 shows how rocks can be moulded to make a rock garden consisting of a pool 19, hollow rocks, 20, 20 whose recesses may be filled with earth and a rock 21 with holes which go all the way through thus giving the plants a better chance to grow right out of the rocks.

Another method producing an irregular surface on pottery is shown in Figures 17 and 18. A piece of sheet metal 22 is set up and soil 12 in clumps of irregular shape piled against this sheet metal to a certain level. The cementitious matter 17 is then poured on the other side of the sheet metal to a level A—A and the sheet 22 is pulled out before it has a chance to set, which permits the cement 17 to run into the cavities between the clumps as shown in Figure 18. This sheet metal 22 can have any irregular shape as shown in Figure 19. This sheet 22 can also be set up on a slant under any angle as shown in Figure 20. The method of pouring materials in this way has the advantage that rocks can be made of fairly predetermined shape by always using the same sheet metal. It also has the additional advantage that rocks can be piled up on a slant as shown in Figure 20 which is not possible with the previous methods that I have described.

Instead of a piece of sheet metal, I can use any other material like paper or cloth. A piece of cloth has the additional advantage that it can be put up very irregularly. When pulled out, after the cementitious material is poured, it makes a very irregular surface.

Figures 22 and 23 show how round pots can be made by having a cylindrical shell 23 set up. The soil 12, 12 is piled against the shell and around it. A core 24 can be set up on the inside and then the cementitious material poured around the core. After it is poured the sheet iron shell 24 is removed which gives a garden pot as shown in Figure 23.

The introduction of soil material into the top of the cementitious mixture after it is poured is not restricted to aerated concrete, but can also be used with ordinary heavy concrete, if this is made wet enough so that the soil material can be pushed in.

The soil material employed in my process may have a higher or a lower specific gravity than the cementitious material, or it may be of the same specific gravity, it being sufficient that at least a portion of the soil material be below the surface of the cementitious material during the setting, or hardening, process.

For the rock material, Portland cement is the most suitable material where the rocks are exposed to the weather. Colors can be added to the cement so that rocks can be produced in any shade or color the same as ordinary concrete. For the same rock different colors can be used so that marble like effects can be obtained. Of course other cementitious materials can also be used such as gypsum, magnesite cement, et cetera, and the rocks made of these materials would be suitable for indoor use.

In order to save rock material the rocks can be

cast hollow. All these materials can be aerated by any suitable method, so as to make the rock material porous and light in weight.

It is evident that larger pieces of rock, bird baths, pools can be suitably reinforced with steel-bars or wire netting in order to make them stronger and light.

I do not limit myself to the particular size, shape, number, arrangement or material of parts as shown and described as these are given simply as a means for clearly describing my invention.

What I claim is:

1. In a process for the production of cementitious masses, the steps which comprise forming a mould from soil, pouring concrete into said mould, placing a plurality of clumps of material upon the surface of said concrete before it has hardened, at least a portion of said clumps being below the surface of said concrete and removing said material by means of water after said concrete has hardened.

2. In a process for the production of cementitious masses, the steps which comprise forming a mould from soil and having an irregular inner face, pouring a cementitious material into said mould, placing a plurality of clumps of soil upon the surface of said cementitious material before it has hardened, at least a portion of said clumps being below the surface of said cementitious material and removing said placed soil from said cementitious material after said cementitious material has hardened.

3. In a process for the production of cementitious masses, the steps which comprise forming a mould from soil, placing a second mould within the first mentioned mould, pouring a cementitious material between the two said moulds, placing a plurality of clumps of soil upon the surface of said cementitious material, at least a portion of said clumps being below the surface of said cementitious material, allowing said cementitious material to harden and removing said moulds from said hardened cementitious material.

4. In a process for the production of cementitious masses, the steps which comprise forming a mould from a material which will practically unchange the liquid contents of a cementitious material placed therein, pouring a cementitious material into said mould, placing a plurality of clumps of removable material which will practically unchange the liquid contents of said cementitious material upon the surface of said cementitious material before it has hardened, at least a portion of said clumps being below the surface of said cementitious material and removing said material after said cementitious material has hardened.

5. In a process for the production of cementitious masses, the steps which comprise depositing clumps of soil of a nature which will practically unchange the liquid contents of a cementitious material, against one side of a thin sheet form, pouring cementitious material against the other side of said form, removing said form before said cementitious material has hardened, allowing said cementitious material to set and removing said soil from said hardened cementitious material.

6. In a process for the production of cementitious masses, the steps which comprise depositing clumps of soil of a nature which will practically unchange the liquid contents of a cementitious material, against one side of a thin sheet form, pouring cementitious material against the other side of said form, removing said form be-

fore said cementitious material has hardened, placing a plurality of clumps of a soil of a nature which will practically unchange the liquid contents of said cementitious material upon the surface of said cementitious material, at least a portion of said clumps being below the surface of said cementitious material, allowing said cementitious material to set and removing said soil from said hardened cementitious material.

7. In a process for the production of cementitious masses, the steps which comprise depositing clumps of soil of a nature which will practically unchange the liquid contents of a cementitious material against a hollow mould open at the bottom, placing a second mould within said first mould, pouring a cementitious material between said moulds, removing said first mentioned mould before said cementitious material has hardened, allowing said cementitious material to fill the interstices of said soil clumps, allowing said cementitious material to harden and removing said soil from said hardened cementitious material.

8. In a process for the production of cementitious masses, the steps which comprise forming a mould having an inner face formed by the inwardly exposed surfaces of an assemblage of clods of soil of irregular shape and unequal size thereby providing a mould surface having abrupt projections with intervening abrupt depressions, pouring a cementitious material into said mould, and removing said mould by disintegrating the soil thereof after said cementitious material has hardened thereby to remove such soil from the complemental pockets formed in the cementitious mass by the mould projections.

9. In a process for the production of cementitious masses, the steps which comprise forming a mould having an inner face formed by the inwardly exposed surfaces of lumps of yieldable plastic material of irregular shape and unequal size which will provide a mould surface having abrupt projections with intervening abrupt depressions, pouring a cementitious material into said mould, and removing said mould after the cementitious material has hardened by causing the plastic material of the mould to yield out of the complemental pockets formed in the cementitious mass by the mould projections.

10. In a process for the production of cementitious masses, the steps which comprise pouring a cementitious material into an open top mould, placing a plurality of clods of soil of irregular shape and unequal size upon the surface of said cementitious material before it has hardened to be there exposed with at least a portion of said clods below the surface of said cementitious material, and removing said placed clods by disintegrating the soil thereof after said cementitious material has hardened thereby to remove such soil from the complemental pockets formed in the surface of the cementitious mass by said clods.

11. In a process for the production of cementitious masses, the steps which comprise pouring a cementitious material into an open top mould, placing a plurality of lumps of yieldable plastic material of irregular shape and unequal size upon the surface of said cementitious material before it has hardened to be there exposed with at least a portion of said lumps below the surface of said cementitious material, and removing said lumps after the cementitious material has hardened by causing the plastic material of said lumps to yield out of the complemental pockets formed in the surface of the cementitious mass by said lumps.

12. In a process for the production of cementitious masses, the steps which comprise forming an open top mould having an inner face formed by the inwardly exposed surfaces of an assemblage of clods of soil of irregular shape and unequal size thereby providing a mould surface having abrupt projections with intervening abrupt depressions, pouring a cementitious material into said mould, placing a plurality of clods of soil of irregular shape and unequal size upon the surface of said cementitious material before it has hardened to be there exposed with at least a portion of said placed clods below the surface of said cementitious material, and removing said mould and said placed clods by disintegrating the soil thereof after said cementitious material has hardened thereby to remove such soil from the complemental pockets formed in the cementitious mass by the mould projections and by said placed clods.
13. In a process for the production of cementitious masses, the steps which comprise forming an open top mould having an inner face formed by the inwardly exposed surfaces of lumps of yieldable plastic material of irregular shape and unequal size which will provide a mould surface having abrupt projections with intervening abrupt depressions, pouring a cementitious material into said mould, placing a plurality of lumps of yieldable plastic material of irregular shape and unequal size upon the surface of said cementitious material before it has hardened to be there exposed with at least a portion of said placed lumps below the surface of said cementitious material, and removing said mould and said placed lumps after the cementitious material has hardened by causing the plastic material of the mould and of said placed lumps to yield out of the complemental pockets formed in the cementitious mass by the mould projections and by said placed lumps.

ERNEST WALTER.